

# United States Patent [19]

Kojima et al.

[11] Patent Number: 4,682,465

[45] Date of Patent: Jul. 28, 1987

[54] FALSE-TWIST TEXTURED YARN OF POLYAMIDE

[75] Inventors: Teiyo Kojima; Heiichiro Matsuda; Masaru Tokizane, all of Otsu, Japan

[73] Assignee: Toray Industries, Inc., Tokyo, Japan

[21] Appl. No.: 679,305

[22] Filed: Dec. 7, 1984

[30] Foreign Application Priority Data

Dec. 7, 1983 [JP] Japan ..... 58-229936

[51] Int. Cl.<sup>4</sup> ..... D02G 3/02

[52] U.S. Cl. ..... 57/247

[58] Field of Search ..... 57/243, 246, 247

[56] References Cited

U.S. PATENT DOCUMENTS

- |           |         |              |       |          |
|-----------|---------|--------------|-------|----------|
| 2,295,593 | 9/1942  | Miles        | ..... | 57/247   |
| 2,771,733 | 11/1956 | Leath et al. | ..... | 57/247   |
| 2,796,655 | 6/1957  | Stuewer      | ..... | 57/247 X |
| 3,651,633 | 3/1972  | Steinmiller  | ..... | 57/247   |
| 3,698,178 | 10/1972 | Iwoka et al. | ..... | 57/247 X |
| 3,939,637 | 2/1976  | Franz et al. | ..... | 57/247   |
| 3,995,420 | 12/1976 | Ohse et al.  | ..... | 57/247   |

Primary Examiner—Donald Watkins

Attorney, Agent, or Firm—Austin R. Miller

[57]

## ABSTRACT

A false-twist textured yarn composed of a polyamide filament yarn excellent in stretchability and heat durability suitable for sports wear is proposed, which is characterized in that the maximum value  $F$  (g) of a shrinkage force under dry heat and a heat treatment temperature  $T$  ( $^{\circ}$ C.), at which the maximum shrinkage force value  $F$  is attained, are defined by the following equations:

$$0.20 \text{ g}/D \geq F/D \geq 0.08 \text{ g}/D \text{ and}$$

$$T_m \geq T \geq T_m - 25$$

wherein  $D$  is the titre of the textured yarn represented by denier, and  $T_m$  is the melt-breakage temperature of the polyamide filament yarn represented by  $^{\circ}$ C., and that the crimp recovery CR of the yarn is 15% or more. The textured yarn is preferably produced from a preoriented undrawn polyamide filament under specific false-twist texturing conditions by means of an in-draw texturing machine with the specific yarn guide for facilitating a threading operation.

5 Claims, 7 Drawing Figures



Fig. 1



Fig. 2A



Fig. 2B



Fig. 3



Fig. 4A



Fig. 4B



Fig. 5



## FALSE-TWIST TEXTURED YARN OF POLYAMIDE

### BACKGROUND OF THE INVENTION

#### 1. Field of the Invention

The present invention relates to a false-twist textured yarn of a polyamide and a method and an apparatus for the production thereof. More particularly, the present invention relates to a false-twisted textured yarn of a polyamide having a high crimp development ability and being excellent in the heat durability and a reasonable method and apparatus for the production thereof.

#### 2. Description of the Related Arts

False-twist textured yarns of polyamides have been known from old, and they are superior to false-twist textured yarns of polyesters and other polymers in the stretchability and they are widely used for the production of woven and knitted stretch fabrics. However, with increase of the grade of sports wears, requirements for stretch materials become severer and presently available false-twist textured yarns of polyamides hardly satisfy these requirements. In the field of clothes for which an especially high stretchability is required, a false-twist textured yarn of a polyamide is mix-woven or mix-knitted with a polyurethane yarn. This, however, results in increase of the manufacturing cost.

In one of methods for obtaining a high-stretch yarn without using a polyurethane yarn, two single yarns to which primary twists have been imparted are doubled, the doubled yarn is strongly twisted in the direction reverse to the direction of the initial twists, the twisted yarn is thermally set and the yarn is then detwisted so that the detwist number is substantially equal to the number of the final twists (see Japanese Examined Patent Publication (Kokoku) No. 33-6699).

A yarn having a high stretchability can be obtained according to this method. However, this method is defective in that the processing steps are complicated and the manufacturing cost becomes high.

There has been proposed another method in which a preoriented undrawn yarn (POY) is false-twisted with a large false-twist number (see Japanese Unexamined Patent Publication (Kokai) No. 50-42152). Though the manufacturing cost can be reduced in this method as compared with that in the former method, the stretchability of the obtained textured yarn is lower than that of the textured yarn obtained according to the former method, because high twists cannot be given to the POY.

For producing a false-twist textured yarn of polyamide at a high speed, there is widely adopted an in-draw texturing system in which a preoriented undrawn yarn (POY) is false-twisted simultaneously with drawing. In fact, when a friction type twister is utilized in this system, the processing speed is as high as 600 to 1000 m/min. On the other hand, the spinning speed of POY is going to reach at a level of 3000 to 4000 m/min. However, the recent needs for higher productivity require further increase of both the false-twist texturing speed and the spinning speed of POY. Various problems should be solved before attaining this object. One of these problems is how to avoid occurrence of fluffs in a false-twisted textured yarn with increase of the false-twist texturing speed. This disadvantage becomes particularly serious when POY spun at a high spinning speed is utilized. The reason is presumed to be that the elongation of POY is reduced with increase of the spin-

ning speed thereof. Moreover, if the titre of the yarn is increased, generation of fluffs becomes conspicuous. The reason is that if the titre is increased, the difference of the yarn length between the inner and outer layers of the yarn is increased and therefore, the outer layer of the yarn is strongly elongated and finally broken to readily cause fluffs.

The length of a yarn path in a false-twist texturing machine tends to be increased with the increase of the texturing speed and now reaches 4 to 5 m or more. Because of the limitation of the ceiling height in a mill, it is difficult to form such a long yarn path linearly in the vertical direction. Accordingly, as shown in FIG. 3, a false-twist texturing machine in which a primary heater 2 and a cooling device 3 are obliquely arranged is often adopted at the present. In view of the facility of the threading operation, it is preferred that a first feed roller 1 and a twister 4 be arranged within the reach of operator's hands. Therefore, a considerable distance more than 50 cm is produced between the first feed roller 1 and the entrance of the primary heater 2 and ballooning of the yarn tends to occur at that area. To prevent occurrence of ballooning of the yarn, a rotary type twist stopping member called "vane tensor" as shown in FIG. 4 is disposed in the vicinity of the entrance of the primary heater 2. However, this rotary member has a drawback to increase formation of fluffs in the resultant false-twist textured yarn.

As pointed out hereinbefore, formation of fluffs in a false-twist textured yarn is aggravated by any of the following false-twist texturing conditions:

- (1) High speed processing.
- (2) Usage of POY spun at a high spinning speed.
- (3) Usage of a yarn of a large titre.
- (4) Usage of a false-twist texturing machine in which the distance between the first feed roller and the entrance of the primary heater is large.

Namely, according to any of the conventional techniques, it is difficult to perform the false-twist texturing operation of POY and obtain a desired textured yarn having a titre of more than 30 denier at a processing speed of at least 600 m/min and a draw ratio lower than 1.35 by using a false-twist texturing machine in which the distance between the first feed roller and the entrance of the primary heater is 50 cm or more.

There has been proposed a method in which instead of the above-mentioned rotary twist stopping member, yarn guide elements for forming a bending yarn path are disposed between the primary heater and the first feed roller to reduce the twist ascent to the first feed roller (see Japanese Examined Patent Publication (Kokoku) No. 53-7976). According to this method, formation of fluffs and reduction of the strength are prevented (such the drawbacks are thought to be caused by partial drawing of the yarn and deformation of the yarn section at the nip point of the first feed roller), but the capacity of inhibiting the twist ascent is poor and this method is not suitable for attaining the object of the present invention. It is considered that, to enhance the capacity of inhibiting the twist ascent by this method, the number of yarn guide elements must be increased for further bending of the yarn path. However, this causes the increase of the resistance to the running yarn as well as the difficulty of the smooth threading operation.

There has been proposed still another method in which a satin-plated bar guide for bending the yarn path between the heater and the feed roller is disposed in the

non-rotary state 200 to 450 mm before the ordinary yarn path and the yarn is half wrapped on this bar guide and turned back (see Japaense Examined Patent Publication (Kokoku) No. 58-48649). According to this method, the distance of the yarn path between the feed roller and the heater is prolonged by turning-back of the yarn, whereby uneven distribution of twists is prevented, causing the decrease of fluffs in the resultant yarn. However, this bar guide has no function of stopping twist ascent and of preventing occurrence of yarn ballooning. Furthermore, in this known method, the yarn tends to be flattened just at the beginning of false-twist texturing and to adhere to the guide. Especially in case of POY, yarn breakage is caused at that time.

A still further method has been proposed in Japanese Unexamined Patent Publication (Kokai) No. 50-42152, for preventing formation of fluffs in the draw-texturing process, in which double twisted portions of at least 3 per cm of yarn length are forcibly formed in a yarn being passing through the twisting zone of the process. This method is effective only when the false-twist texturing speed is as low as about 100 to about 200 m/min, but, at such a high speed as 600 m/min or more, the texturing operation becomes unstable and the yarn breakages is increased.

#### SUMMARY OF THE INVENTION

It is a primary object of the present invention to provide a false-twist textured yarn composed of a continuous polyamide filament yarn, which can be suitably utilized for making a knitted or woven fabric excellent in the stretchability, and a reasonable method and apparatus for the production thereof. More specifically, the present invention provides a false-twist textured yarn having less fluffs even if the false-twist texturing operation is carried out at a high speed by using a false-twist texturing machine having such a yarn path that the distance between the first feed roller and the entrance of the primary heater is 50 cm or more.

In accordance with a first aspect of the present invention, there is provided a false-twist textured yarn composed of a continuous polyamide filament yarn, characterized in that the maximum shrinkage force value  $F$  (g) of the shrinkage force under dry heat and a heat treatment temperature  $T$ , at which the maximum value  $F$  is attained, are defined by the following equations:

$$0.20 \text{ g/d} \geq F/D \geq 0.08 \text{ g/D, and}$$

$$T_m \geq T \geq T_m - 25$$

wherein  $D$  is the titre of the textured yarn represented by denier and  $T_m$  is the melt-breakage temperature of the polyamide filament yarn represented by  $^{\circ}\text{C.}$ , and that the crimp recovery  $CR$  of the yarn is 15% or more.

In accordance with a second aspect of the present invention, there is provided a false-twist textured yarn as set forth above, wherein the textured yarn has a cohesive lubricant agent containing a wax having a high melting point.

In accordance with a third aspect of the present invention, there is provided a method for producing a false-twist textured yarn from a starting continuous polyamide filament yarn by a false-twist texturing machine. The method is characterized in that the birefringence  $\Delta n$  of the starting filament yarn to be fed to the texturing machine, the yarn tension  $t$  (g/d) in a twisting

zone of the texturing machine and the heat setting temperature  $H$  ( $^{\circ}\text{C.}$ ) are defined by the following equations:

$$\Delta n \geq 35 \times 10^{-3},$$

$$0.8 \geq t \geq 0.4, \text{ and}$$

$$H_m - 10 \geq H \geq H_m - 25,$$

wherein  $H_m$  is a melting point ( $^{\circ}\text{C.}$ ) of said filament yarn after it is fully drawn.

In accordance with a fourth aspect of the present invention, there is provided a method for producing a false-twist textured yarn from a preoriented undrawn continuous polyamide filament yarn by a false-twist texturing machine. The filament yarn has a birefringence  $\Delta n$  of at least  $35 \times 10^{-3}$  and is treated with a cohesive lubricant agent containing a wax having a high melting point. The method is characterized in that in-draw texturing system is carried out by utilizing a friction twister of belt nip type under a false-twist condition represented by the following equation:

$$N \cdot \sqrt{D} \geq 28,000,$$

wherein  $N$  is a false twist number ( $t/m$ ) and  $D$  is a total denier of the resultant textured yarn.

In accordance with a fifth aspect of the present invention, there is provided a method for starting the production of a false-twist textured yarn from a preoriented undrawn continuous polyamide multifilament yarn by an in-draw texturing machine. The multifilament yarn has a birefringence in of at least  $35 \times 10^{-3}$  and the in-draw false-twist texturing machine comprises a first feed roller, a primary heater disposed downstream of the former at a point separate by 50 cm or more from the feed roller and means for providing a bending yarn path between the first feed roller and the primary heater by a plurality of yarn guide elements. The method is characterized in that the multifilament yarn is threaded to at least one of said yarn guide elements, disposed upstream of said primary heater within a distance of less than 20 cm, whereby the multifilament yarn is started to travel into the heater and be twisted and heated therein, and thereafter, the multifilament is threaded to the remaining yarn guide elements to form the yarn path bending zigzag with a total wrapping angle around said yarn guide elements being more than 300 degrees.

In accordance with a sixth aspect of the present invention, there is provided a false-twist texturing machine for processing a filament yarn at a high speed, which comprises a first feed roller, a primary heater, a false-twister, a second feed roller and a winding means. The texturing machine is characterized in that two groups A and B of yarn guide elements, the two groups of the yarn guide elements being secured on separate brackets, are disposed upstream of the primary heater in the vicinity of an entrance thereof, and at least one of the brackets is movable toward and apart from the other bracket so that said yarn guide elements on the respective brackets co-operatively constitute a yarn path bending zigzag.

#### BRIEF DESCRIPTION OF THE DRAWINGS

Other objects and advantages of the present invention will be more apparent from the following description

by referring to the attached drawings illustrating preferred embodiments of the present invention, wherein:

FIG. 1 is a graph depicting a relationship between a heat treatment temperature and a shrinkage force of a polyamide filament;

FIG. 2A is a schematic side view of an embodiment of a yarn guide utilized for the present invention, especially for the fifth and sixth aspects thereof;

FIG. 2B is a partially enlarged view of FIG. 2A illustrating an arrangement of yarn guide elements;

FIG. 3 is a schematic side view of a typical in-draw false-twist texturing machine, mainly illustrating a yarn path thereof;

FIGS. 4A and 4B are side and front views of the conventional rotary type twist stopping member, respectively; and

FIG. 5 is a schematic side view of a false-twist texturing machine provided with a belt nip type false-twister.

#### DESCRIPTION OF THE PREFERRED EMBODIMENTS

The present invention will now be described in detail.

In the first aspect of the present invention, the shrinkage force under dry heat is measured by a thermal stress measuring apparatus (Model KE-1 supplied by Kanebo Engineering K.K.) under the following conditions.

Sample length: 20 cm (in a loop form)

Temperature-elevating rate: 120 seconds/300° C.

Initial load: 0.1 g/d

Measurement frequency: 5 times

An example of the measurement is shown in FIG. 1. The maximum value  $F$  (g) of the shrinkage force is determined by reading the apparent maximum value  $F_A$  (g) of the shrinkage force in FIG. 1, subtracting the initial tension  $F_O$  (g) from the read value and dividing the obtained value by two. Namely, the maximum value  $F$  of the shrinkage force under dry heat is expressed by the following formula:

$$F = \frac{1}{2}(F_A - F_O)$$

The heat treatment temperature  $T$  (°C.) is the temperature at which said apparent maximum value  $F_A$  of the shrinkage force is attained, and the melt-breakage temperature  $T_m$  (°C.) is the temperature at which the shrinkage force is zero (see FIG. 1).

The crimp recovery  $CR$  (%) is determined on a sample pretreated under the following conditions according to the test method of JIS L-1090.

(1) An initial load of 2 mg/d per denier is hung down from a small hank of a textured yarn to be tested.

(2) The hank is immersed in hot water maintained at  $98 \pm 1$  °C. for 20 minutes while the initial load is imposed on the hank.

(3) The hank is taken out from hot water and the initial load is removed, and the hank is allowed to stand still in the stationary state for more than about 12 hours so that the hank is not disturbed, whereby the water equilibrium state is attained.

(4) A lighter load of 2 mg/d is applied to the treated hank and then a heavier load of 0.1 g/d is added thereto. The crimp recovery  $CR$  is calculated according to the following formula:

$$CR (\%) = \frac{l - l_1}{l} \times 100$$

wherein  $l$  stands for the length of the hank under the lighter plus heavier loads and  $l_1$  stands for the length of the hank under the lighter load alone.

Nylon-6 and nylon-66 may be used for the continuous polyamide filament yarn in the present invention. The denier and filament number are not particularly critical, but ordinarily, the denier is in the range of from about 10 for stockings to about 400 for industrial materials and the filament number is in the range of from 2 for stockings to 144 for industrial materials.

The first characteristic feature of the present invention resides in that the maximum value  $F$  (g) of the shrinkage force under dry heat is in the range represented by the following equation:

$$0.20D \geq F \geq 0.08D$$

The value  $F$  of a conventional false-twist textured yarn composed of a continuous polyamide filament yarn is smaller than 0.06D. This value  $F$  has a relation to the crimp developing ability, by which the textured yarn can develop its latent crimps in a woven or knitted fabric against the restriction caused by the structure of the woven or knitted fabric. The present inventors made investigations with a view to improve the stretchability of a woven or knitted fabric composed of a false-twist textured yarn of a polyamide, and found that one condition for attaining this object resides in increase of the crimp developing ability of the false-twist textured yarn in a woven or knitted fabric. It also was found that in order to increase this crimp developing ability, it is necessary to increase the value  $F$ . Especially in the case where the false-twist textured yarn is used for a product for which a high stretchability is required, such as tights or a swimming suit, the value  $F$  should be at least 0.08D. However, if the value  $F$  is excessively large, a problem of a poor dimensional stability arises. Accordingly, it is indispensable that the value  $F$  should be up to 0.20D.

The second characteristic feature of the present invention resides in that the heat treatment temperature  $T$  (°C.) at which the maximum value  $F$  (g) of the shrinkage force under dry heat is attained is in the range represented by the following equation:

$$T_m \geq T \geq T_m - 25$$

The temperature  $T$  of a conventional false-twist textured yarn of a polyamide is about  $(T_m - 40)$  and the difference of this temperature  $T$  from the melt-breakage temperature  $T_m$  is large. In contrast, in the false-twist textured polyamide yarn of the present invention, the difference between  $T$  and  $T_m$  is small. The value of  $T_m$  is substantially constant for one polymer. Accordingly, if the kind of the polymer is the same, the value  $T$  of the false-twist textured polyamide yarn of the present invention is larger than that of the conventional false-twist textured polyamide yarn. The value  $T$  has an influence on the thermal stability of the false-twist textured yarn, and, therefore, it is apparent the thermal stability of the false-twist textured polyamide yarn according to the present invention is higher than that of the conventional one.

The third characteristic feature of the present invention resides in that the crimp recovery  $CR$  (%) is 15% or more. The  $CR$  value is a measure indicating the degree of crimp, and in order to attain a sufficient stretchability, it is indispensable that this condition should be satisfied. Namely, it is important that the  $CR$

value should be 15% or more while the above-mentioned two requirements are satisfied.

The second aspect of the present invention will now be described.

By the term "wax having a high melting point" is meant a wax having a melting point higher than 90° C. Examples thereof are polyethylene wax, polypropylene wax, oxidized paraffin wax and microcrystalline wax. It is indispensable that the wax should be incorporated in the cohesive lubricant agent in an amount of at least 3%, preferably at least 8% by weight. Of course, an emulsifier and an antistatic agent may be incorporated in the lubricant agent in addition to the wax. In order to improve the adhering property of the wax, a mineral oil may be incorporated in the lubricant agent.

The cohesive lubricant agent containing the wax having high melting point should be applied when a preoriented undrawn polyamide filament yarn is melt-spun. The wax is present on the surface of the preoriented undrawn yarn and exerts a function of bonding the respective filaments to one another. By the subsequent false-twist texturing processing, this bonding among the filaments are released and the wax component is allowed to flow appropriately, which enhances mutual slip among the filaments after texturized and improves a stretchability of the resultant yarn. If the wax is applied after the false-twist texturing, the bonding among the filaments is not released, and the touch of the resulting knitted or woven fabric becomes rough and hard and the stretchability is not improved. The wax component should have a high melting point exceeding 90° C. The reason is that the residual ratio of the wax component after scouring or washing is influenced by the melting point. Namely, if a wax having a melting point lower than 90° C., such as paraffin wax or ester type wax, is used, the wax residual ratio after scouring becomes very low.

The third aspect of the present invention will now be described.

A false-twist texturing machine comprising feed rollers, a heat treating device, a false-twister and a winder may be used in this aspect. A false-twister in which the ratio of the detwisting tension to the twisting tension can be set to less than 1.2 is preferably used. In this connection, a pin type false-twister is not preferred. It is indispensable that a continuous filament yarn of a polyamide to be fed in the present invention should have a birefringence  $\Delta n$  of at least  $35 \times 10^{-3}$ . The method of the present invention can be carried out by processing a fully drawn yarn by means of a conventional false-twist texturing machine or by processing an undrawn yarn, especially POY, by means of an in-draw false-twist texturing machine.

In the present invention, the yarn tension  $t$  (g/d) should be adjusted within the range represented by the following equation:

$$0.8 \geq t \geq 0.4$$

The value  $t$  within the above-mentioned range is much larger than that adopted in the conventional false-twist texturing method. According to the conventional technique, the value  $t$  is ordinarily 0.1 to 0.12 in case of the pin-type false-twister and does not exceed 0.4 even in case of the friction-type false-twister. In general, increase of the twisting tension results in increase of the detwisting tension and reduction of the crimp recovery. Therefore, it has been considered that the twisting tension should be reduced as low as possible provided the

processing stability is maintained. The requirement of  $0.8 \geq t \geq 0.4$  is contrary to this conventional concept. However, if this requirement is combined with the requirement of the heat setting temperature  $H$  described hereinafter, a special effect not heretofore expected can be attained.

In the method for producing a false-twist textured polyamide yarn according to the present invention, the heat setting temperature  $H$  should be adjusted within 10 the range represented by the following equation:

$$H_m - 10 \geq H \geq H_m - 25$$

wherein  $H_m$  stands for the melting point (°C.) of the 15 continuous polyamide filament yarn after it is fully drawn.

The value  $H$  customarily adopted in the conventional 20 false-twist texturing method does not exceed the level of  $(H_m - 30)$ . The heat setting temperature  $H$  corresponds to the surface temperature of a heater of a false-twist texturing machine. If the heater temperature is excessively elevated, fusion bonding is caused among 25 filaments and the appearance and crimp characteristics of the resultant textured yarn are degraded. In the conventional concept, it has been considered that an ordinary 30 textured yarn cannot be obtained if the heater temperature is higher than  $(H_m - 25)$ . The requirement of  $H_m - 10 \geq H \geq H_m - 25$  according to the present invention is contrary to the generally accepted concept.

If one of the yarn tension requirement of  $0.8 \geq t \geq 0.4$  and the heat setting temperature requirement of  $H_m - 10 \geq H \geq H_m - 25$  is satisfied alone, only a textured yarn having a low crimp recovery and/or an appearance degraded by fusion bonding is obtained. To 35 our great surprise, it was found that when both of the above-mentioned requirements are simultaneously satisfied, a false-twist textured yarn free of fusion bonding or low crimp recovery can be obtained. The present invention has been completed based on this finding. In the method of the present invention, there is not any limitation of the false-twist texturing speed or the like, other than the above-mentioned requirements. However, especially excellent effects can be attained when the processing speed is 600 to 1000 m/min.

The cohesive lubricant agent containing a high-melting point wax, which is used in the fourth aspect of the 40 present invention, is the same as the wax-containing lubricant agent described hereinbefore with respect to the second aspect of the present invention. In the fourth aspect of the present invention, it is preferred that the birefringence  $\Delta n$  of the starting preoriented undrawn polyamide filament yarn (POY) be at least  $35 \times 10^{-3}$ . The nip-type friction twister used in the method of the 45 present invention comprises a pair of elements such as belts, discs or rollers arranged to confront each other, and the yarn passing between the paired elements is gripped from both the sides by the elements and the yarn is twisted and propelled by the action of the elements.

In the present invention, the relation represented by 50 the following equation should be established between the false twist number  $N$  and the denier  $D$  of the false-twist textured yarn:

$$N \cdot \sqrt{D} \geq 28,000$$

It is well-known that the crimp size of a textured yarn decreases with increase of the false twist number. If this value is smaller than 28,000, crimps are coarse and an intended high stretchability cannot be obtained.

In the present invention, a false-twist texturing machine provided with a belt-nip-type friction twister is preferably utilized. The reason is that this type of the twister gives not only a twisting action but also propelling action to a yarn as same as a disc type friction twister consisting of three rotating axes and is hence suitable for high speed false-twist texturing. Further, the belt-nip-type twister has an excellent yarn-gripping ability, which is important to the present invention. Namely, in order to satisfactorily texture an undrawn polyamide filament yarn treated with the cohesive lubricant agent containing the high-melting-point wax with a high false twist number matching with the requirement of  $N \cdot D \geq 28,000$ , it is necessary to use a twister having a high yarn-gripping ability. From this viewpoint, use of a belt-nip-type friction twister is significant. Also, a preoriented undrawn yarn is suitably utilized due to its easy twistability. In the present invention, a known draw ratio may optionally be adopted in the in-draw texturing process without any limitation.

The fifth and sixth aspects of the present invention will now be described with reference to embodiments illustrated in the accompanying drawings.

FIG. 2A shows the vicinity of an entrance of a primary heater of the high-speed false-twist texturing machine of the present invention.

A movable bracket 12 to which guide elements B1 and B2 are attached is located at a right lower position indicated by a dot line, and in this state, threading, travelling and false-twisting of the yarn at the starting period are carried out. Then, the movable bracket 12 is moved to a left upper position indicated by a solid line. At this point, the bracket 12 intersects a bracket 11, on which other guide elements A1 and A2 are attached. Accordingly, the yarn is travelled along a bent yarn path formed by the guide elements A2, B2, A1 and B1.

The entire structure of the false-twist texturing machine is illustrated in FIG. 3. A yarn Y taken out from a yarn drum passes through a first feed roller 1, a primary heater 2, a cooling device 3, a false-twister 4 and a second feed roller 5 and is wound as a cheese 6. During this travel, the yarn Y is heated, twisted, cooled and detwisted, and thus a false-twist textured yarn is formed. A secondary heater and a third feed roller may be disposed subsequently to the second feed roller. In case of the false-twist texturing machine having the above-mentioned yarn path, a twist stopping member 7 is disposed between the first feed roller 1 and the entrance of the first heater 2 to prevent occurrence of ballooning due to the twist ascent from the twisting zone to the first feed roller 1. The twist stopping member according to the present invention will now be described with reference to FIG. 2B. The twist stopping member consists of a plurality of yarn guide elements A1, A2, B1 and B2, each of which may be of the stationary type or of the rotary type forcibly rotated by running of the yarn. It is preferred that the guide elements be formed of a hard metal or ceramic having a smooth surface.

As the ceramic, alumina, titanium and zirconia types are preferred, and the surface roughness is preferably smaller than 04S. The guide elements preferably have a drum-like shape with a groove of U-shaped cross-section. Further the diameter of the guide element corre-

sponding to a yarn contact portion is preferably about 8 to about 15 mm.

The distance between the entrance of the primary heater 2 and the yarn guide element A2 closest thereto should be less than 20 cm. If this distance exceeds 20 cm, a balloon of the yarn is formed and the intended twist stopping function cannot be exerted. It is preferable that the distance between the adjacent guide elements, B1 and A1, A1 and B2 or B2 and A2 along the 10 yarn path (precisely, the distance between the points where the yarn separates from a surface of each guide element) is also less than 20 cm. If this distance exceeds 20 cm, the influence of a balloon of the yarn cannot be neglected. FIG. 2B illustrates the yarn path after attaining 15 the steady state of the false-twisting operation. The yarn is sequentially engaged with the yarn guide element B1, A1, B2 and A2 at wrapping angles  $\theta_1$ ,  $\theta_2$ ,  $\theta_3$  and  $\theta_4$ , respectively. The total wrapping angle of  $\theta_1 + \theta_2 + \theta_3 + \theta_4$  should be more than 300 degrees. If 20 the total wrapping angle is less than 300 degrees, the twist stopping effect becomes insufficient. On the contrary, if the total wrapping angle is too large, the resistance to the running yarn is increased and uneven drawing is caused. Accordingly, it is preferable that the total 25 wrapping angle is less than 450 degrees. Furthermore, it is preferable that the wrapping angle of the upstream side guide element is always larger than that of the downstream side guide element and vice versa, so that the relation of  $\theta_1 > \theta_2 > \theta_3 > \theta_4$  is established.

30 In the case where the threading operation is carried out by using the above-mentioned yarn guide element, as shown in FIG. 3, the yarn Y taken out from the package is firstly nipped on the second feed roller 5 while the end of the yarn is being sucked by a suction 35 pipe (not shown), whereby travelling of the yarn is started, and then, the yarn is sequentially engaged with the false-twister 4, the cooling device 3 and the primary heater 1 and is then engaged with the yarn guide elements A1, A2, B1 and B3 so that the total wrapping 40 angle becomes more than 300 degrees. Then, the yarn end sucked by the suction pipe is transferred to the package 6 to start winding. In this method, it is preferable that the timing of nipping the yarn on the first feed roller 1 is preferably set just before or after the time 45 when the yarn is engaged with the yarn guide elements.

In the above-mentioned threading operation, the total wrapping angle of more than 300 degrees should be attained after the travelling, twisting and heating of the yarn have been started. If the travelling, twisting and 50 heating operations are started after formation of the total wrapping angle of more than 300 degrees, the frictional resistance to the yarn caused by the yarn guide elements becomes excessive to cause a yarn breakage and the threading operation cannot be performed smoothly. This is because non-twisted POY falls in contact, in the flattened state, with a circumference of the yarn guide elements corresponding to the wrapping angle of more than 300 degrees, and the friction coefficient therebetween is extremely increased. In addition to this, at the moment of yarn starting while 55 keeping the yarn in contacting with the surfaces of the yarn guide elements, a static frictional force is imposed on the yarn from the guide elements, which also exerts an excessive travelling resistance to the yarn.

60 In order to carry out the above-mentioned threading operations more smoothly, the yarn guide elements A1 and A2 are attached to a stationary bracket 11 and the yarn guide elements B1 and B2 are attached to a mov-

able bracket 12. At the initial stage of the threading operation, the movable bracket 12 is retreated to the position indicated by a dot line in FIG. 2A, and after travelling and twisting of the yarn are started, the movable bracket 12 is moved toward the stationary bracket 11 to contact the yarn with the primary heater 2, whereby heating is started. The movable bracket 12 is further advanced so that the yarn guide elements B<sub>1</sub> and B<sub>2</sub> form a zigzag yarn path in co-operation with the yarn guide elements A<sub>1</sub> and A<sub>2</sub> on the bracket 11, and the total wrapping angle of  $\theta_1 + \theta_2 + \theta_3 + \theta_4$  amounts to more than 300 degrees. In this case, though the function of causing the yarn to fall in contact with the primary heater and the function of forming the total wrapping angle of more than 300 degrees are both achieved by the movement of the movable bracket 12, the former function may be accomplished by another means irrelevant to the movable brackets.

One effect of the false-twisted textured yarn composed of the continuous polyamide filament yarn according to the first aspect of the present invention is that a fabric product obtained by using this textured yarn is excellent in the stretch characteristics.

It is apparent that a knitted or woven fabric being sufficiently shrinkable at the dyeing step becomes a dyed fabric having a high stretchability. Since the false-twist textured yarn of the present invention has a very large maximum value F of shrinkage force, and the fabric made thereof can be sufficiently shrunk against the tension imposed in the dyeing step or the frictional restriction force acting between the adjacent yarns in the fabric structure, a fabricated product having a high stretchability can be obtained. This product is excellent in stiffness (anti-drape). A fabric made of the conventional false-twist texturing yarn tends to largely reduce its stretchability during dyeing and heat setting. However, a fabric made of the yarn according to the present invention is improved in this regards and the stretchability thereof can be maintained for a long time even after the post heat treatment. Especially, the yarn according to the present invention is advantageous when it is mix-knitted with a non-stretch yarn such as cotton yarn or acrylic spun yarn for the production of socks, training wears and sports wears, because the false-twist textured yarn of the present invention can compensate the low resiliency of the non-stretch yarn due to its sufficient stretchability.

The effect of the false-twist textured polyamide yarn according to the second aspect of the present invention is that a highly stretchable textured yarn, any properties of which are hardly changed by scouring, washing or the like can be obtained.

One advantage of the method for producing a false-twist textured polyamide yarn according to the third aspect of the present invention is that the method can be carried out without any substantial change being made to the existing apparatus. Another advantage is that limitations to be imposed on increase of the processing speed are not serious. In general, as the processing speed is increased, the yarn tends to vibrate at respective parts of the yarn path to cause a so-called ballooning due to the increase of rotating speed and the processing stability is disturbed. Accordingly, in the conventional process, for avoiding this disadvantage at the high-speed false-twist texturing, the twisting tension is increased to restrict occurrence of ballooning. However, if the twisting tension is excessively increased in the conventional technique, the crimp ratio of the resul-

tant textured yarn becomes poor. In contrast, according to the method of the present invention, the twisting tension t is higher compared to the conventional method and therefore, the texturing processing can be performed stably at a high speed without ballooning.

One advantage of the fourth aspect of the present invention is that a highly stretchable textured yarn can be obtained simply by controlling the spinning and false-twist texturing steps. In short, the complicated twisting step of a low efficiency, that is indispensable in the conventional technique, is not necessary.

Another advantage of the fourth aspect is that a highly stretchable textured yarn can be produced at a high speed as the same level as the processing speed adopted in the conventional in-draw false-twist texturing method.

Still another advantage of the fourth aspect is that the kind and the type of the polymer, the denier and the filament number of the starting yarn are not substantially limited. The method of the fourth aspect can be applied to a variety of preoriented undrawn polyamide filament yarns that can be false-twisted.

The effect attained by the fifth and sixth aspects of the present invention is that the in-draw texturing process can be started stably and a high-quality false-twist textured yarn free of fluffs can be obtained even if the processing speed is increased. The abovesaid effect is particularly excellent when highly oriented POY having a large denier is used. The method of these aspects can be carried out only by remodelling the entrance portion of the primary heater of the false twist texturing machine and changing the procedures of the threading operation, which does not need large expense for remodelling.

According to the apparatus of the sixth aspect of the present invention, the operation of forming a necessary yarn wrapping angle to the yarn guide elements in the midway of the threading operation can be easily performed, especially when the movable bracket is constituted to be operated with a lever from the floor level, which operation, usually, must be performed at an elevated position and needs a considerable time. Moreover, further advantage is that an excessive space is not necessary for the apparatus because it can be easily provided by remodelling the existing false-twist texturing machine.

The features of the present invention will now be more apparent with reference to the following examples that by no means limit the scope of the invention.

#### EXAMPLE 1

A nylon-6 chip was melted according to the ordinary method, spun at a spinning speed of 5200 m/min and directly wound on a drum to obtain a preoriented undrawn yarn (POY) having a denier of 89 and a filament number of 24. The birefringence in of this POY was  $39 \times 10^{-3}$ . The melting point of a drawn yarn obtained by fully drawing this POY was 217°C. The POY was fed to an in-draw false-twist texturing machine (MACH CRIMPER 333-II supplied by Murata Kikai K.K.), and various false-twist textured yarns were prepared by changing the processing speed, heat setting temperature and twisting tension as indicated in Table 1. The titre, strength (g/d), elongation (%), crimp recovery (%), maximum value F (g), heat treatment temperature T (°C.) providing the maximum value of the shrinkage force and melt-breakage temperature T<sub>m</sub> (°C.) of each

of the obtained false-twist textured yarns are listed in Table 2.

Interlock knitted fabrics were prepared by using these false-twist textured yarns and were then dyed. With respect to each fabric, the stretchability in the wale direction, the appearance and the stiffness were evaluated. The obtained results are listed in Table 2. The stretchability was determined according to the following test procedures:

(1) Three test pieces having a width along the course direction of 5 cm and a length along the wale direction of about 30 cm were collected from the sample fabric.

(2) By using a constant-speed stretching tensile tester

TABLE 1-continued

| Run No. | Conditions for Production of False-Twist Textured Yarns |                          |                                |                        |                   |
|---------|---------------------------------------------------------|--------------------------|--------------------------------|------------------------|-------------------|
|         | Processing Speed (m/min)                                | False Twist Number (T/m) | Heat Setting Temperature (°C.) | Twisting Tension (g/d) | Remarks           |
| 9       | 800                                                     | 3400                     | 205                            | 0.50                   | present invention |
| 10      | 1000                                                    | 3400                     | 185                            | 0.70                   | comparison        |
| 11      | 1000                                                    | 3400                     | 195                            | 0.67                   | present invention |
| 12      | 1000                                                    | 3400                     | 205                            | 0.63                   | present invention |

TABLE 2

| Run No. | Titre (denier) | Strength (g/d) | Elongation (%) | Properties of False-Twist Textured Yarns and Knitted Fabrics |       |         |          | Stretchability (%) | Appearance of Knitted Fabric | Stiffness    |
|---------|----------------|----------------|----------------|--------------------------------------------------------------|-------|---------|----------|--------------------|------------------------------|--------------|
|         |                |                |                | CR (%)                                                       | F (g) | T (°C.) | Tm (°C.) |                    |                              |              |
| 1       | 72.0           | 5.65           | 27.5           | 28.4                                                         | 3.1   | 165     | 206      | 42                 | good                         | good         |
| 2       |                |                |                | not evaluated because of extreme fused bonding               |       |         |          |                    |                              |              |
| 3       |                |                |                | not evaluated because of extreme fused bonding               |       |         |          |                    |                              |              |
| 4       | 70.2           | 5.60           | 26.8           | 26.8                                                         | 6.0   | 162     | 207      | 35                 | slightly bad                 | slightly bad |
| 5       | 70.0           | 5.50           | 26.2           | 29.6                                                         | 5.7   | 182     | 206      | 50                 | good                         | good         |
| 6       | 70.3           | 5.10           | 24.0           | 32.5                                                         | 6.1   | 188     | 207      | 56                 | good                         | excellent    |
| 7       | 68.4           | 5.63           | 27.0           | 22.1                                                         | 7.3   | 161     | 205      | 33                 | between slightly bad and bad | slightly bad |
| 8       | 68.3           | 5.47           | 27.1           | 24.3                                                         | 7.5   | 183     | 206      | 48                 | good                         | good         |
| 9       | 68.3           | 5.25           | 24.2           | 26.7                                                         | 7.0   | 186     | 205      | 53                 | good                         | good         |
| 10      | 66.3           | 5.65           | 25.0           | 15.5                                                         | 9.1   | 162     | 204      | 31                 | bad                          | bad          |
| 11      | 66.4           | 5.60           | 23.8           | 16.3                                                         | 8.8   | 184     | 207      | 47                 | good                         | good         |
| 12      | 66.5           | 5.45           | 22.9           | 18.3                                                         | 9.0   | 184     | 205      | 50                 | good                         | good         |

provided with an automatic recorder, the test piece was grasped at the opposite ends thereof by a pair of grips of the tester at a grip distance of 20 cm, under an initial load corresponding to the same weight as that of the sample fabric having a size of 5 cm x 1 m.

(3) The test piece was stretched at a pulling speed of 20 cm/min to the point of 18 kg wt., and the grip distance was measured to the order of  $\frac{1}{2}$  mm. The stretchability (%) was calculated according to the following formula:

$$\text{stretchability (\%)} = \frac{l_1 - l}{l} \times 100$$

wherein  $l$  stands for the initial grip distance

(mm) and  $l_1$  stands for the grip distance measured when stretched to the point of 1.8 kg.

The mean value from three test pieces was listed in Table 2 (calculated down to the first decimal place).

From the results shown in Table 2, it will readily be understood that the false-twist textured yarn of the present invention is excellent in the stretchability, the appearance of the knitted fabric and the stiffness.

## EXAMPLE 2

35 A nylon-6 polymer was melted according to the ordinary method and was spun at a spinning speed of 4000 m/min to obtain a POY having a denier of 87.2 and a filament number 24. An oiling agent was applied, during the spinning process, to the yarn so that the oil content of the yarn becomes 0.6 weight %. The melting point and residual ratio of the wax component used in the oiling agent are shown in Table 3.

40 The residual ratio referred to herein is an index indicating the durability of the wax component, which is determined according to the following method: a 200-cc beaker is charged with 150 cc of warm water heated at 60° C., and 5 g of a sample yarn is immersed in water and ultrasonic washing is carried out for 5 minutes. The washed sample is dehydrated by a spin dryer so that the water content is reduced to 50%. Then, the sample is air-dried. The amount of the wax left in the dried sample and the amount of the wax contained in 5 g of the sample before the washing treatment are measured, and the residual ratio is calculated according to the following formula:

$$\text{Residual ratio (\%)} = \frac{\text{amount of wax in sample after washing}}{\text{amount of wax in sample before washing}} \times 100$$

55 60 The so-obtained POY was fed to the false-twist texturing machine provided with the belt nip type friction twister, shown in FIG. 5, and the yarn was subjected to the false-twist texturing under conditions shown in Table 4. The properties of the obtained false-twist textured yarn are shown in Table 5.

65 The crimp recovery CR was determined according to the method described hereinbefore.

TABLE 1

| Run No. | Conditions for Production of False-Twist Textured Yarns |                          |                                |                        |                   |
|---------|---------------------------------------------------------|--------------------------|--------------------------------|------------------------|-------------------|
|         | Processing Speed (m/min)                                | False Twist Number (T/m) | Heat Setting Temperature (°C.) | Twisting Tension (g/d) | Remarks           |
| 1       | 400                                                     | 3400                     | 185                            | 0.21                   | comparison        |
| 2       | 400                                                     | 3400                     | 195                            | 0.24                   | comparison        |
| 3       | 400                                                     | 3400                     | 205                            | 0.22                   | comparison        |
| 4       | 600                                                     | 3400                     | 185                            | 0.43                   | comparison        |
| 5       | 600                                                     | 3400                     | 195                            | 0.46                   | present invention |
| 6       | 600                                                     | 3400                     | 205                            | 0.45                   | present invention |
| 7       | 800                                                     | 3400                     | 185                            | 0.56                   | comparison        |
| 8       | 800                                                     | 3400                     | 195                            | 0.53                   | present invention |

The crimp developing ability CCT (g) was determined by using a continuous crimp tester (CCT) supplied by Rothchild Co., under the following conditions:

Yarn speed: 16 m/min

Initial tension: 0.1 g/d

Overfeed ratio: 4 to 8%

Heater temperature: 150° C.

From the results shown in Table 5, it will readily be understood that false-twist textured yarns Nos. 2, 3, 4, 5, 6 and 7 according to the method of the present invention are excellent in both the crimp recovery CR and the crimp developing ability CCT. When these textured yarns were knitted into interlock knitted fabrics of 28G and the stretchability thereof in the wale direction were measured, it was found that a high stretchability of 50 to 60% was obtained in case of the false-twist textured yarns obtained according to the method of the present invention, while the stretchability was as low as 30 to 35% in case of comparative textured yarns.

TABLE 3

| Oiling Agents Used |                       |                                     |                    |
|--------------------|-----------------------|-------------------------------------|--------------------|
| Oiling Agent No.   | Wax Component         | Melting Point (°C) of Wax Component | Residual Ratio (%) |
| 1                  | polyethylene wax      | 103                                 | 89                 |
| 2                  | oxidized paraffin wax | 92                                  | 70                 |
| 3                  | paraffin wax          | 60                                  | 9                  |
| 4                  | not added             | —                                   | —                  |

TABLE 4

| False-Twist Texturing Conditions |                                          |                             |
|----------------------------------|------------------------------------------|-----------------------------|
| Processing Level                 | Belt Crossing Angle (degrees) of Twister | Belt Speed/Processing Speed |
| A                                | 110                                      | 1.35                        |
| B                                | 110                                      | 1.50                        |
| C                                | 120                                      | 1.45                        |
| D                                | 120                                      | 1.60                        |
| E                                | 130                                      | 1.65                        |
| F                                | 130                                      | 1.80                        |

False-twist texturing processing speed: 600 m/min

Heater temperature: 185° C.

Draw ratio: 1.844

TABLE 5

| Results of False-Twist Texturing Processing |                  |                  |                          |                      |                        |        |         |                   |
|---------------------------------------------|------------------|------------------|--------------------------|----------------------|------------------------|--------|---------|-------------------|
| Run No.                                     | Oiling Agent No. | Processing Level | False Twist Number (T/m) | Twisting Tension (g) | Detwisting Tension (g) | CR (%) | CCT (g) | Remarks           |
| 1                                           | 1                | A                | 3290                     | 24                   | 31                     | 46.7   | 2.45    | comparison        |
| 2                                           | 1                | B                | 3450                     | 28                   | 16                     | 51.0   | 2.60    | present invention |
| 3                                           | 1                | C                | 3610                     | 23                   | 35                     | 55.9   | 2.75    | present invention |
| 4                                           | 1                | D                | 3720                     | 25                   | 28                     | 57.3   | 2.80    | present invention |
| 5                                           | 1                | E                | 3880                     | 22                   | 26                     | 58.6   | 2.90    | present invention |
| 6                                           | 1                | F                | 4060                     | 26                   | 14                     | 58.3   | 2.90    | present invention |
| 7                                           | 2                | D                | 3740                     | 27                   | 29                     | 54.5   | 2.65    | present invention |
| 8                                           | 3                | D                | 3730                     | 27                   | 28                     | 45.4   | 2.45    | comparison        |
| 9                                           | 4                | D                | 3780                     | 26                   | 30                     | 44.1   | 2.40    | comparison        |

Incidentally, the belt nip type friction twister used in Example 2 was as shown in FIG. 5. The tension of the feed yarn Y supplied from a spool 21 was adjusted by the tension compensator 22, and then, the yarn Y was heated and false-twisted between the feed roller 23 and delivery roller 26. Namely, the running yarn Y was false-twisted by the crossing belts 25 and was simultaneously heated by the heater 24, whereby the false-twist texturing processing was accomplished. Then, the yarn

60 The test was carried out in the same manner as in Example 3 while fixing the twisting tension to 25 g and changing the number of yarn guide elements, the distance between the entrance of the primary heater and the nearest yarn guide element, the distance between the adjacent yarn guide elements and the total wrapping angle as indicated in Table 7. Other conditions were the same as in Example 3. The test results are listed in Table 7. In Run No. 1, the yarn was wound on only one yarn guide element at a total wrapping angle of 360 degrees.

Y was fed out by the delivery roller 26 and wound in a package 28 by the winding drum 27.

In the foregoing embodiment, another delivery roller may be arranged subsequently to the delivery roller 26, and known process such as filament entanglement or filament looping may be carried out between the two delivery rollers.

## EXAMPLE 3

10 A POY (natural draw ratio of 1.33) of nylon-6 spun at a spinning speed of 5200 m/min, having a denier of 70 (after drawing at a draw ratio of 1.28) and a filament number of 24, was subjected to the false-twist texturing at a processing speed of 600 m/m, a primary heater temperature of 185° C. and a false twist number of 3390 T/m by using the draw-texturing machine shown in FIGS. 2 and 3. The twist stopping systems shown in Table 6 were alternatively utilized. The draw ratio was slightly increased or decreased from a standard value of 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050

In this case, many fluffs were formed and the threading operation was difficult. In Run Nos. 2 through 14, fluffs were hardly formed and the threading operation could be performed smoothly. However, when the distance between the primary heater and the nearest yarn guide element was larger than 200 mm, ballooning was caused and the processing became unstable (Run No. 7). Similar undesirable results were obtained when the distance between the adjacent yarn guide elements was larger than 200 mm (Run No. 10) and when the wrapping angle was less than 300 degrees (Run No. 11).

In conclusion, Run Nos. 2 to 6, 8, 9, 12, 13 and 14 satisfying the conditions of the present invention represented a desired results.

$0.20 g/D \geq F/D \geq 0.08 g/D$ , and

$T_m \geq T \geq T_m - 25$

5 wherein D is the titre of the textured yarn represented by denier, and  $T_m$  is the melt-breakage temperature of said polyamide filament represented by  $^{\circ}\text{C}$ . and that the crimp recovery CR of the yarn is 15% or more.

2. A false-twist textured yarn according to claim 1, wherein said polyamide is one selected from the group comprising nylon 6 and nylon 66.

3. A false-twist textured yarn according to claim 1, wherein said filament yarn is a multi-filament yarn.

TABLE 7

| Run No. | Number of Yarn Guide Elements | Distance (mm) between Entrance of Primary Heater and Yarn Guide Element | Distance (mm) between Yarn Guide Elements | Total Wrapping Angle (degrees) | Test Results                  |            |                     |                   |
|---------|-------------------------------|-------------------------------------------------------------------------|-------------------------------------------|--------------------------------|-------------------------------|------------|---------------------|-------------------|
|         |                               |                                                                         |                                           |                                | Number (per 2000 m) of Fluffs | Ballooning | Threading Operation | Remarks           |
| 1       | 1                             | 120                                                                     | 40                                        | 360                            | 37                            | not caused | difficult           | comparison        |
| 2       | 2                             | 120                                                                     | 40                                        | 360                            | 2.0                           | not caused | easy                | present invention |
| 3       | 4                             | 120                                                                     | 40                                        | 360                            | 0                             | not caused | easy                | present invention |
| 4       | 5                             | 120                                                                     | 40                                        | 360                            | 0.1                           | not caused | easy                | present invention |
| 5       | 4                             | 50                                                                      | 40                                        | 360                            | 0                             | not caused | easy                | present invention |
| 6       | 4                             | 190                                                                     | 40                                        | 360                            | 0                             | slight     | easy                | present invention |
| 7       | 4                             | 220                                                                     | 40                                        | 360                            | 0.2                           | caused     | easy                | comparison        |
| 8       | 4                             | 120                                                                     | 60                                        | 360                            | 0                             | not caused | easy                | present invention |
| 9       | 4                             | 120                                                                     | 190                                       | 360                            | 0.1                           | slight     | easy                | present invention |
| 10      | 4                             | 120                                                                     | 220                                       | 360                            | 0.2                           | caused     | easy                | comparison        |
| 11      | 4                             | 120                                                                     | 40                                        | 270                            | 0                             | prominent  | easy                | comparison        |
| 12      | 4                             | 120                                                                     | 40                                        | 300                            | 0                             | slight     | easy                | present invention |
| 13      | 4                             | 120                                                                     | 40                                        | 310                            | 0.1                           | slight     | easy                | present invention |
| 14      | 4                             | 120                                                                     | 40                                        | 450                            | 0.3                           | not caused | slightly difficult  | present invention |

We claim:

1. A false-twist textured yarn composed of a continuous polyamide filament yarn, characterized in that the maximum value F (g) of the shrinkage force under dry heat and a heat treatment temperature T ( $^{\circ}\text{C}$ ), at which said maximum shrinkage force value F is attained, are defined by the following equations:

40 4. A false-twist textured yarn according to claim 1, wherein the titre of said filament yarn is in a range of from 10 denier to 400 denier and the filament number thereof is in a range of from 2 to 144.

5. A false-twist textured yarn according to claim 1, wherein said textured yarn has a cohesive lubricant agent containing a wax having a high melting point.

\* \* \* \* \*